

Patented Apr. 8, 1924.

1,489,357

# UNITED STATES PATENT OFFICE.

WILLIAM J. McELROY, OF NEW YORK, AND JOHN CLARKE, OF MANHASSET, NEW YORK,  
ASSIGNORS TO ALCHEMIC GOLD COMPANY, INC., A CORPORATION OF NEW YORK.

## PRINTING INK.

No Drawing.

Application filed July 25, 1922. Serial No. 577,429.

*To all whom it may concern:*

Be it known that we, WILLIAM J. McELROY, a citizen of the United States, and a resident of the borough of Manhattan, city, 5 county, and State of New York, and JOHN CLARKE, a citizen of the United States, and a resident of the village of Manhasset, town of North Hempstead, county of Nassau, and State of New York, have invented a new and 10 useful Improvement in Printing Inks, of which the following is a description, as well as of the manner and process of making, constructing, compounding, and using the same, in such full, clear, concise, and exact 15 terms as to enable any person skilled in the art or science to which it appertains or with which it is most nearly connected to make, construct, compound, and use the same.

Our invention relates generally to printing 20 inks and particularly to those having metallic powders as their pigments.

The objects of our invention are the production of improved printing inks adapted for general use and more especially for use 25 in embossing and die-printing upon book-cloth, leather and other materials commonly used for book-casings; particular objects are the production of inks of this class which shall be adapted for application by a heated 30 die, plate or other impression member, pre-heated to embossing temperatures, and which shall be characterized by the qualities of drying immediately under the relatively high temperatures preferred in embossing 35 metallic powders; and having properties of strongly adhering to and covering smoothly, evenly and completely the surface upon which they are stamped; of being rendered lustrous by the heat of the metal by which 40 they are impressed upon such object; of permanently retaining their original color and luster without tarnishing or fading; of high boiling point and of low volatility.

Further objects are the provision of an 45 ink with the foregoing qualities which can be mixed ready for use by the manufacturer and which will not corrode or otherwise deteriorate in the container, and which, when packaged, and transported shall remain in 50 its original state with its qualities and both its physical and chemical conditions unimpaired even after long lapse of time.

Our present invention consists in the discovery that printing inks such as set forth 55 in our Patent No. 1,450,692, may attain the

desired attributes above recited, particularly as to covering and luster qualities to a highly superior degree by employing as the metallic pigment to be mixed with the highly viscous vehicle described, a mixture of bronze powders, such mixture being composed of bronze powder of the fineness customarily employed in making inks, namely, that exemplified by the grade known commercially as "Hemmerdinger's Special No. 1," to which has been 60 added a more comminuted powder exemplified by the grade known generally in the trade as "lining." We have further discovered that with such composite powder, the heavy-bodied pigment vehicles referred to in our 65 aforesaid patent, and whose composition is hereinafter exemplified, combine to make an ink in which the powdered metallic pigment, by virtue of the amount thereof in a state of fine subdivision, and by virtue of the high 70 viscosity of the vehicle, will tend to remain in suspension as long as the ink is fluid. 75

The stamped or embossed or printed impression obtained with this ink affords a more intense pigmentation, and, when dried, is more pliable than that obtainable either with the coarser particles used alone or with the finer particles used alone. This is apparently because the former leaves microscopic interstices between the particles, while the latter produces too smooth or flat a surface to reflect light in the manner the coarser individual particles do when present, hence the desired "glance" or brilliance of luster is lacking. The best results are attained by 80 the use of the two grades in substantially those relative proportions hereinafter exemplified. 85

As an example of the preferred proportions of the ingredients named, we take, by 95 weight,

95 per cent terpineol and

5 per cent rosin oil, and stir until thoroughly mixed.

With 84 per cent of this mixture we incorporate 16 per cent of powdered cumarone resin, e. g., that known under the trade name of "Cumar," and warm this mixture upon a water-bath at 100° centigrade, stirring meanwhile, until the "Cumar" is thoroughly 100 dissolved, which will result in about 20 minutes with vigorous stirring. The batch is 105 then allowed to cool. From this batch we take one-third and add thereto two-thirds of bronze powder, both by weight. This mix. 110

ture is then stirred until the bronze powder is thoroughly and evenly incorporated. The ink resulting is of pasty and semi-fluid consistency, similar to that of printing inks generally.

As the metallic pigment above intended, we prefer a mixture of bronze powder of the grade known commercially as Hemmerdinger's Special No. 1, with 80 per cent of 10 which is mixed 20 per cent of the finer grade of bronze powders known generally in the trade as "lining," a more finely comminuted species of such powders, such species being that produced in the process of 15 usual manufacture of bronze powders by air-floating from the mill those particles which have been reduced to the state of subdivision of fine, almost impalpable, dust.

The proportions above exemplified may be 20 varied somewhat without appreciable variation of the product.

While thus specifying terpineol and rosin oil as the constituents preferred of our binder solvent vehicle, we wish to be understood as typifying thereby a binder vehicle having the desired properties as such, first, of an active solvent of the synthetic resins named; second, as of the desired body adapted to maintain the bronze powders in sustained suspension; third, as of the requisite degree of volatility to be driven off by the temperature used in embossing metallic pigments to impart the desired luster thereto; fourth, affording that degree of plasticity and elasticity to the impression which will prevent its cracking; fifth, the necessary neutrality which will preserve the metallic particles from corrosion on standing when mixed in ink form; sixth, which shall not cause the impressed characters to tarnish; and seventh, which shall be colorless or of such color as will not detract from the desired metallic luster. Within the limitations imposed by these criteria, the binder vehicle 30 may be any of the suitable solvents or combinations thereof. This printing composition is primarily intended for printing book covers which, when of cloth, are prepared as cases with a strong coating of glue to hold 40 the cloth to the backing. As the boiling point of the vehicle specified is approximately 428° Fahrenheit, the impression temperature must suffice to drive off the volatile solvent, that the impression may be dry, but 50 must not be so high as to draw the glue through the cloth and thereby cause blisters in the impression or darken it. Preferably,

therefore, the described composition should be used as an ink at a temperature substantially that of the boiling point of the solvent 60 vehicle. As will be obvious, however, the ink set forth may be used at lower temperatures, or cold, and the impression artificially dried thereafter,

By virtue of the comparatively high specific gravity of the synthetic resins produced as condensation products of naphtha, and the heavy body of the solvent therefor herein named, the solution obtained affords an especially valuable vehicle for the metallic 70 pigments in that the tendency of the bronze powder to settle is checked and a persistent suspension thereof is attained.

Having thus described the preferred embodiment of our invention and the best 75 method now known to us of producing and usefully applying same, we claim:

1. A printing composition comprising a finely divided metallic pigment consisting of a mixture of the less fine grade of bronze 80 powders with a substantial quantity of the finer grade of bronze powders resultant from re-grinding the former grade added thereto, a neutral binder, a viscous solvent for said binder of low volatility, the dissolved binder 85 constituting a vehicle for the pigment of such viscosity that the pigment tends to remain in suspension therein.

2. A printing composition comprising a binder, a highly viscous solvent therefor of 90 low volatility and a powdered metallic pigment consisting of a mixture of bronze powders of two grades of fineness, the quantity ratio between the grades being substantially four of one grade to one of the finer grade 95 by weight, the latter grade being of the fineness of "linings."

3. A printing ink containing a metallic pigment consisting in part of bronze powders of the grade known as "linings," such 100 part substantially exceeding the percentage of this grade normally present in bronze powders which have not been subject to air floating.

4. A printing ink composition containing 105 a metallic pigment comprising a mixture of bronze powders of two grades of fineness, as follows: 80 per cent of a grade coarser than that identified as "lining" and 20 per cent of "lining," "Cumar," and a solvent for said 110 "Cumar" adapted to maintain the metallic pigment in suspension.

WILLIAM J. McELROY.  
JOHN CLARKE.